

## UNITED STATES PATENT OFFICE.

ALICE MARION HART, OF LONDON, ENGLAND, ASSIGNOR, BY MESNE ASSIGNMENTS,  
TO EDMUND R. CUMMINS, OF WORCESTER, MASSACHUSETTS.

## PRODUCTION OF CARBON.

No Drawing.

Application filed July 7, 1922. Serial No. 573,479.

*To all whom it may concern:*

Be it known that I, ALICE MARION HART, a subject of the King of Great Britain, residing at London, England, have invented 5 certain new and useful Improvements in and Relating to the Production of Carbon, of which the following is a specification.

This invention is for improvements in the production of carbon, and has particular 10 reference to the carbonization of peat, lignite, sawdust and such like, and of waste materials, such as the refuse of cotton, paper and rice husking mills, straw, dead leaves, river suds, and non-mucilaginous seaweed, 15 as for example the *Poseidonia australis*.

According to the present invention the material to be carbonized is, if necessary, ground into a coarse powder, and is impregnated with a weak solution of a metallic salt and is then roasted on a hot plate 20 to carbonization, while freely exposed to the air. The salts utilizable are sodium carbonate, sulphate, chloride or acetate, and the corresponding potassium salts; sodium, 25 or potassium phosphate, ferrous sulphate and calcium chloride. As a general rule it will be found that the salt may be used in relatively quite small proportions and permits of carbonization in the open air without 30 out appreciable production of ash. That is to say the addition of the salt prevents combustion of the material and thus permits carbonization to be carried on with full access of air. If the salt were not added, 35 combustion would obviously take place.

For example, in carrying this invention into effect dried peat, ground or disintegrated, as may be required, is moistened throughout with a 1 per cent solution of 40 sodium carbonate (or soda crystals) in approximately the proportion of one half pint to a pint of solution to one pound of the dry peat and the mass so impregnated is roasted on a hot plate with access of air until completely 45 carbonized.

Wet peat may be carbonized in a similar manner. In this case no added water is required, the metallic salt in the proportion of about 0.25 per cent, is dissolved in the least 50 possible amount of water, and is intimately mixed with the peat by an appropriate method of disintegration. The process of carbonization is the same as that described above.

Alternatively weak solutions of a ferrous sulphate, or one of the salts already mentioned, may be used, care being taken, in reference to the use to which the carbon is to be put, that the salt employed should be one which will either not be detrimental or 60 can be easily removed.

In the case where a pure carbon is required it should be boiled in a dilute solution of hydrochloric acid, for instance a 1 per cent solution and then dried. The ash 65 can thus be reduced to under 1 per cent and consists chiefly of calcium chloride, and silica.

The carbon produced may be directly worked up into briquettes for furnace fuel, 70 in which case it is important to select a binder which carbonizes and does not vaporize with heat.

It has been found that by the process herein set forth materials such as peat or 75 sawdust can be readily and economically carbonized and carbon obtained in good yield.

I claim:

1. A process of carbonizing carbon containing materials, for the production of carbon, consisting in treating the materials to be carbonized with a metallic salt of a nature to prevent immediate combustion of the material but permit carbonization there- 80 under heat, and then subjecting the mass to heat in the presence of air.

2. A process of carbonizing carbon containing materials, for the production of carbon, consisting in impregnating the materials to be carbonized with a weak solution of a metallic salt of such nature as to prevent immediate combustion of the material but permit carbonization thereof under heat, 85 and then roasting the mass while freely exposed to air.

3. A process of carbonizing carbon containing materials, for the production of carbon, consisting in impregnating the materials to be treated with a weak solution of 100 a metallic salt of a character to prevent immediate combustion of the material while permitting carbonization thereof under heat, and then roasting same on a hot plate while freely exposed to air.

4. A process of carbonizing carbon-containing material for the production of carbon, consisting in moistening said material 105

with a solution of a sodium salt and roasting same while exposed to the air, until complete carbonization takes place.

5. A process of carbonizing carbon-containing materials, such as peat, lignite, sawdust, suds, and the like, for the production of carbon, consisting in intimately distributing throughout the mass of material to be carbonized a metallic salt of such nature 10 that it prevents immediate combustion of the material while permitting the carbonization of the same under heat, and then subjecting the mass while in the presence of air to sufficient heat to carbonize it.

15. 6. A process of carbonizing dried peat for the production of carbon consisting in disintegrating said peat, moistening same with a 1 per cent solution of sodium carbonate in the proportion of one half to one pint of 20 solution to one pound of dried peat, and roasting the resultant mass on a hot plate with access of air until completely carbonized.

7. A process of carbonizing wet peat for 25 the production of carbon, consisting in adding to said wet peat a metallic salt in the proportion of about 0.25 per cent, dissolved

in the least possible quantity of water, the metallic salt being in the nature to prevent immediate combustion of the material but 30 permit carbonization thereof under heat, intimately mixing the solution with the peat, and roasting the same on a hot plate while freely exposed to the air.

8. A process of carbonizing carbon-containing materials such as peat, lignite, sawdust, suds and the like for the production of carbon consisting in treating said materials with a weak solution of ferrous sulphate, and roasting the mass in the presence of air. 35

9. A process of carbonizing carbon-containing materials such as peat, lignite, sawdust, suds and the like for the production of pure carbon, consisting in treating said materials with a weak solution of a metallic salt roasting the mass in the presence of air 40 until completely carbonized, boiling the carbonized mass in a dilute solution of hydrochloric acid, and finally drying the resultant product. 45

In testimony whereof I have signed my name to this specification.

ALICE MARION HART.